

H. BRUMMETT & W. H. COLBATH.  
INNERSOLE MATERIAL AND PROCESS OF MAKING THE SAME.  
APPLICATION FILED JULY 11, 1916.

1,204,844.

Patented Nov. 14, 1916.

Fig. 1.



Fig. 2.



Inventors.  
Howard Brummett  
William H Colbath  
by Heard Smith & Tenant  
Atty's.

# UNITED STATES PATENT OFFICE.

HOWARD BRUMMETT AND WILLIAM H. COLBATH, OF NATICK, MASSACHUSETTS,  
ASSIGNORS OF ONE-THIRD TO GEORGE A. SPEAR, OF MEDFORD, MASSACHUSETTS.

## INNERSOLE MATERIAL AND PROCESS OF MAKING THE SAME.

1,204,844.

Specification of Letters Patent. Patented Nov. 14, 1916.

Application filed July 11, 1916. Serial No. 108,725.

*To all whom it may concern:*

Be it known that we, HOWARD BRUMMETT and WILLIAM H. COLBATH, both citizens of the United States, residing at Natick, county 5 of Middlesex, State of Massachusetts, have invented an Improvement in Innersole Materials and Processes of Making the Same, of which the following description is a specification.

10 This invention relates to the composition of a new material in sheet form for use in inner soles for shoes and to the process of producing such material.

15 The material which is in sheet form is particularly designed to be cut up into inner soles for shoes of the McKay, standard screw, or nailed type wherein the inner sole and other superimposed parts of the shoe are united together by through and through 20 stitching, by standard screws, or by nails or pegs.

25 The object of the invention is to produce a material which shall be tough, flexible, sweat and waterproof, which shall not be subject to decay or deterioration, which shall securely hold the thread, screws, nails or pegs employed in the manufacture of the shoes, and which shall produce a cheap and satisfactory inner sole.

30 The invention resides in a material in sheet form and in the process of making the same in which the main constituents are wool fiber and crude asphalt commingled when the asphalt is heated into liquid form 35 and in which after the commingled fiber and asphalt have been reduced by pressure to sheet form the exterior surfaces of the material are coated with paint to give a finished coating of the required color, and 40 finally coated with a waxy substance.

The invention also resides in a material of this character which is built up when required of a plurality of sheets of the said material cemented together by a cement having asphalt as its identifying constituent.

45 The nature of the invention will appear more fully from the accompanying description and drawings and it will be particularly defined in the claims.

In the drawings Figure 1 is a perspective 50 view of an inner sole embodying the invention; Fig. 2 is a detail enlarged of a portion of a cross-section of the material forming the inner sole and embodying one form of the invention.

55 In carrying out the invention and forming the material wool fiber and crude asphalt are employed as the main constituents. The wool fiber may be such as usually constitutes waste material. Wool fiber is preferably employed but a certain proportion, say up to about one-third of cotton fiber may be mixed with the wool fiber and has been found satisfactory.

60 The term "fiber" as hereafter used herein 65 is therefore to be understood as comprising wool fiber or the aforesaid mixture of wool and cotton fiber or any fiber having similar characteristics to those of wool fiber or to a mixture of wool and cotton fiber, where 70 the latter constitutes one-third or less of the mixture. The asphalt employed is the crude asphalt of commerce.

75 The first step in the process consists in commingling the fiber and the crude asphalt which is done by heating the asphalt to a sufficiently liquid condition to enable the fiber to be thoroughly mixed therewith. This is accomplished by stirring or working 80 the fiber into the hot liquid asphalt. We have found that one part of asphalt to three and one-half parts of wool fiber by weight produces a suitable mixture, but this may be varied within reasonable limits.

85 The next step in the process consists in forming the resultant mixture into sheet form by subjecting it to pressure while warm. This may be carried out by passing the heavy viscous mixture between rolls until it is reduced to a thin sheet. If machines of sufficient strength, and exerting sufficient pressure are available the resulting sheet may be of the total thickness required for the inner sole material. If as more probable less powerful machines are 90 available, the resultant sheet may be thinner so that the total thickness of the required sheet of inner sole material will be composed 95

of or built up from, as hereinafter set forth, two or more of the thin sheets of material.

The next step of the process consists in drying the sheet material after it is reduced 5 to sheet form. For this purpose the sheet material may be simply left standing at ordinary room temperature until it is dry and hard.

The next step of the process consists in 10 coating both surfaces of the sheet material with paint. For this purpose ordinary commercial paint may be used and any required color may be employed.

In case the required thickness of sheet material is obtained by building up a plurality, that is, two or more thin sheets, then the next step in the process consists in coating the surfaces to be juxtaposed of a plurality 15 of sheets of said material with a cement 20 having as its essential constituent asphalt. We have found that a very satisfactory cement for this purpose is produced by mixing 7½ pounds of asphalt, 4 ounces linseed oil and 1 quart turpentine, but these proportions 25 may be varied within a reasonable extent and gasoline may be employed in place of turpentine.

If the preceding step is employed the next 30 step of the process consists in drying the cement coating of the cement coated sheets which again may be performed by allowing the sheets to stand at room temperature until the cement is dry.

If the preceding two steps are employed 35 then the next step in the process consists in heating the cement coated surfaces until the cement is rendered tacky or sticky.

If the preceding three steps in the process are employed then the next step consists 40 in bringing into juxtaposition the tacky cement coated surfaces of a sufficient plurality of said sheets to give the required total thickness of material.

If the preceding four steps of the process 45 are employed then the next step in the process consists in subjecting the juxtaposed sheets to pressure which may be done by passing them between pressure rollers.

In case the preceding five steps of the 50 process are employed, then the next step in the process consists in drying the built up sheet. This may be done by allowing it to stand at room temperature until it is dry and hard.

The final step in the process in each case 55 consists in finishing the painted exterior surfaces of the sheet, whether of one thickness or resulting from building up two or more sheets, with a coating of waxy substance.

This coating is for the purpose of keeping 60 the finished sheets from adhering together, and it also acts to facilitate the passage of the needle in the stitching operation to clean

the needle and to wax the thread, and when screws and nails are used to assist in their 65 passage into the material. For this coating we prefer to use paraffin or carnauba wax, but any similar waxy material may be employed.

Having fully described our invention, 70 what we claim as new and desire to secure by Letters Patent is:

1. The process of making sheet material for inner soles for shoes which consists in commingling fiber and hot liquid crude asphalt forming the resultant mixture into sheet form by subjecting it to pressure while hot, drying the sheet material, coating the exterior surfaces with paint, and coating the painted surfaces with a waxy substance. 80

2. The process of making sheet material for inner soles for shoes which consists in commingling fiber and hot liquid crude asphalt, forming the resultant mixture into sheet form by subjecting it to pressure while 85 warm, drying the sheet material, coating both surfaces of said material with paint, coating the surfaces to be juxtaposed of a plurality of sheets of said material with a cement containing asphalt, drying the coated 90 sheets, heating the cement coated surfaces until the cement is rendered tacky, bringing into juxtaposition the tacky cement coated surfaces of a sufficient plurality of said sheets to give the required total thickness of 95 material presenting painted surfaces at the exterior, subjecting the juxtaposed sheets to pressure and finishing the painted exterior surfaces of the resultant built up sheet with a coating of waxy substance. 100

3. The process of making sheet material for inner soles for shoes which consists in commingling fiber and hot liquid crude asphalt, forming the resultant mixture into sheet form by subjecting it to pressure 105 while warm, drying the sheet material, coating the surfaces to be juxtaposed of a plurality of sheets of said material with a cement containing asphalt, drying the coated sheets, heating the cement coated 110 surfaces until the cement is rendered tacky, bringing into juxtaposition the tacky cement coated surfaces of a sufficient plurality of said sheets to give the required total thickness of the material, and subjecting the juxtaposed sheets to pressure. 115

4. A sheet material for inner soles for shoes composed of fiber and crude asphalt commingled and pressed into sheet form 120 coated with paint and finished with a waxy coating.

5. A sheet material for inner soles for shoes composed of a plurality of juxtaposed compressed sheets of commingled fiber and crude asphalt having their juxtaposed surfaces secured together by a cement contain- 125

ing asphalt, and having the exterior surfaces coated with paint and with an outer dressing of waxy substance.

6. A sheet material for inner soles for  
5 shoes composed of a plurality of juxtaposed  
compressed sheets of commingled fiber and  
crude asphalt having their juxtaposed sur-

faces secured together by a cement containing asphalt and with the exterior surfaces coated with paint.

In testimony whereof, we have signed our names to this specification.

HOWARD BRUMMETT.  
WILLIAM H. COLBATH.